

## UNITED STATES PATENT OFFICE

2,225,339

PRECIPITATION HARDENED COPPER  
ALLOY

Richards H. Harrington, Schenectady, N. Y., assignor to General Electric Company, a corporation of New York

No Drawing. Application September 12, 1936,  
Serial No. 100,561

4 Claims. (Cl. 148—11.5)

The present invention relates to precipitation hardened copper alloys and more particularly to a process for improving the properties of copper-chromium-beryllium alloys. An alloy of this 5 composition is disclosed in the patent to Dahl 1,847,929 and contains about 0.1% to 1% beryllium, about 0.4% to 6% chromium, with the remainder copper. The alloy disclosed in the patent is age or precipitation hardened by heating it to an elevated temperature, quenching and reheating to an intermediate temperature. When precipitation hardened, this alloy is relatively soft and I have found that its properties 10 may be improved by cold working and also by cold working followed by an additional heat treatment.

If cast rods about 1 $\frac{1}{4}$  inches thick and containing 0.4% chromium, 0.1% beryllium, and about 99.5% copper are precipitation hardened 15 in the usual manner, for example, by heating for about one hour at 900° C., quenching in water, cold swaging to 1 inch diameter and then reheating to 475° C. for an hour the following properties are obtained:

20 Tensile strength..... 47,700 lbs./sq. in.  
Proportional limit..... 30,000 lbs./sq. in.  
Elongation..... 27%  
Hardness..... 63 Rockwell B.  
Electrical conductivity..... 71% that of copper

The structure obtained in the cast rod by the above process is characterized by the presence of the usual slip bands which are present in substantially all cold worked alloys. Also the 25 room temperature physical properties of the alloy are relatively unaffected by reheating up to about 400° C. and recooling.

I have found that if the 1 $\frac{1}{4}$  inch rods of the above noted composition are heated for about one 30 hour at a temperature of 900° C., quenched in water, then reheated at 500° C. for one hour, air cooled and then swaged to 1 inch diameter the following properties are obtained:

35 Tensile strength..... 49,400 lb./sq. in.  
Proportional limit..... 35,200 lbs./sq. in.  
Elongation..... 12%  
Hardness..... 70 Rockwell B.  
Electrical conductivity..... 67% that of copper

40 Cold working after precipitation hardening, it will be observed, effects a marked increase in tensile strength, proportional limit and hardness. Furthermore, the resulting product is characterized by a comparative freedom from the 45 slip bands ordinarily expected in cold worked

material. It is understood, of course, that cold working can also be accomplished by rolling, forging, etc.

If the material thus produced is now reheated 5 at about 100° C. for about 1 $\frac{1}{2}$  hours and air cooled, the following properties are obtained:

|                              |                         |
|------------------------------|-------------------------|
| Tensile strength.....        | 50,600 lbs./sq. in.     |
| Proportional limit.....      | 35,300 lbs./sq. in.     |
| Elongation.....              | 11%                     |
| Hardness.....                | 73 Rockwell B           |
| Electrical conductivity..... | 66.4% of that of copper |

These properties are relatively unaffected by reheating up to about 300° C. and recooling. However, reheating to temperatures about 300° C. 15 results in an increase in electrical conductivity at the expense of lower tensile strength. Reheating to a secondary aging temperature above 400° C. results in properties inferior to those obtained by a single aging followed by cold 20 working.

The specific application of the above alloy obviously will determine which of the above treatments, i. e. (1) precipitation hardening followed by cold working, or (2) precipitation hardening 25 followed respectively by cold working and reheating should be employed. The first treatment is particularly adapted for the production of material to be used in the manufacture of electrical conducting springs while the second process which is in effect a double aging process with intermediate cold working between the first and second reheat is adapted for use where maximum hardness is of importance as in resistance 30 welding electrodes.

What I claim is new and desire to secure by Letters Patent of the United States:

1. The process for improving the properties of precipitation hardened alloys consisting of about 0.1% to 1% beryllium and 0.4% to 6% 40 chromium and the remainder copper, which comprises cold working said precipitation hardened alloy and thereafter aging said alloy.

2. The process for improving the properties of precipitation hardened alloys consisting of 45 about 0.1% to 1% beryllium and 0.4% to 6% chromium and the remainder copper, which comprises cold working said precipitation hardened alloy and thereafter reheating said alloy at a temperature of about 100° C. and cooling. 50

3. The process for improving the properties of a precipitation hardened alloy containing about 0.1% to 1% beryllium, 0.4% to 4% chromium with the remainder copper, which comprises producing a condition of strain in said 55

precipitation hardened alloy by cold working and thereafter aging said alloy, the physical and electrical properties of the alloy thus produced being substantially unaffected by reheating up to about 300° C. and recooling.

5. 4. The process for improving the properties of a precipitation hardened alloy containing about 0.1% to 1% beryllium, 0.4% to 4% chromium

with the remainder copper, which comprises producing a condition of strain in said precipitation hardened alloy by cold working, and thereafter reheating said alloy at a temperature of about 100° C. for about 1½ hours and air cooling from that temperature. 5

RICHARDS H. HARRINGTON.